

Nov. 22, 1927.

1,649,924

F. L. ROMAN ET AL

INSULATED ELECTRICAL CONDUCTOR

Filed Dec. 12. 1925



Inventors  
Frank L. Roman  
Harry T. Winsemius  
by *Halseth*  
ATT'y.

## UNITED STATES PATENT OFFICE.

FRANK LOUIS ROMAN, OF CHICAGO, AND HARRY THOMAS WINSEMIUS, OF CONGRESS PARK, ILLINOIS, ASSIGNORS TO WESTERN ELECTRIC COMPANY, INCORPORATED, OF NEW YORK, N. Y., A CORPORATION OF NEW YORK.

## INSULATED ELECTRICAL CONDUCTOR.

Application filed December 12, 1925. Serial No. 75,011.

This invention relates to insulated electrical conductors, and more particularly to electrical conductors provided with so-called "flame-proof" insulation.

5 The object of the present invention is the provision of an electrical conductor with an inexpensive and efficient flexible covering of flame-proof insulation.

In order to attain this object there is provided in one embodiment of the invention, 10 an electrical conductor in wire form having a coating of suitable insulating enamel covered with a cotton serving impregnated with chlorinated naphthalene to reduce its 15 inflammability, and with an outer braided covering of cotton which is also preferably flame-proofed.

Other objects and features of the invention will be apparent from the following detailed description and the accompanying drawing which shows an insulated wire embodying one form of the invention.

In accomplishing the invention, an electrical conductor such as a tinned copper wire 25 is covered with a fibrous material which is impregnated with a halogenated material such as chlorinated naphthalene. The invention may take a variety of forms, an embodiment of which is shown in the accompanying drawing, in which the numeral 10 refers to a metallic conductor and 11 is a coating of insulating material such as the usual enamel. Over the enamel 11 is placed a serving or servings 12 of textile material, 30 preferably cotton, which is impregnated with chlorinated naphthalene or other halogenated material in a manner which will be described more in detail hereinafter. On the outside of the serving 12 is a flame-proof 35 braided covering 13, preferably braided cotton, which has been treated with ammonium phosphate to decrease its inflammability.

In impregnating the textile covering 12 various types of halogenated material may 40 be employed, but uniformly good results have been obtained in producing an insulated conductor in accordance with this invention by the use of a grade of chlorinated naphthalene which is marketed under the trade name of halowax. In using the chlorinated naphthalene, if a comparatively refined compound is employed, it is preferable 45 that it be mixed with a comparatively small

amount of a bituminous material, preferably refined coal tar, to increase its adhesiveness. 55 Good results are also obtained by employing crude chlorinated naphthalene generally termed crude halowax or halowax pitch and about 5% of refined coal tar. Other types of halogenated materials which may be used 60 in the practice of the invention are bromonaphthalene or other materials related to naphthalene, such as anthracene or coal tar treated with one of the halogens.

After the serving 12 has been placed on 65 the enamel 11 in either a single layer or a plurality of layers, the conductor is passed through a bath of melted halogenated material to obtain a thorough impregnation of the serving. The serving 12 may be silk, 70 cotton or other textile strand, but on account of the lower price of cotton and since it has good electrical insulating characteristics when employed in connection with the present invention, this material is preferred. 75

The insulated conductor may be employed without the braided covering 13, but this covering improves the appearance of the conductor and serves to protect the other insulation from abrasion, and for these reasons 80 in most cases will probably be employed. Any type of braided covering may be used but in its preferred form it consists of braided cotton which has previously been treated with a flame-proofing material such as ammonium phosphate.

An insulated conductor produced according to the present invention is of great value because it is quite resistant to burning, possesses good electrical characteristics, and in 90 addition is economical to manufacture. Another advantage where an enameled conductor is employed, is that the chlorinated material has a tendency to somewhat soften the enamel making it readily removable for the purpose of soldering or otherwise, and at the same time not affecting the insulating value of the enamel. This softening effect of the enamel is not sufficient to in any way dissociate it from the conductor, since it is 100 retained in place by the cotton serving or other insulation, which in the practice of the invention is applied over it. Still another advantage resulting from the use of chlorinated naphthalene is that this material will not interfere with soldering opera- 105

tions should it in any way come in contact with the bare wire which is to be subjected to a soldering operation.

What is claimed is:

5. An insulated wire comprising an electrical conductor having a coating of fibrous material treated with a halogenated material.
10. An insulated wire comprising an electrical conductor having a coating of insulating material treated with a mixture of chlorinated naphthalene and a bituminous material.
15. An insulated wire comprising an electrical conductor having a textile insulating covering impregnated with chlorinated naphthalene.
20. An insulated wire comprising an electrical conductor, a serving of cotton impregnated with a halogenated material, and a braided covering of cotton treated with a flame-proofing material.
5. An insulated wire comprising an electrical conductor, a serving of cotton impregnated with chlorinated naphthalene, and a 25 braided covering of flame-proofed cotton.
6. An insulated wire comprising an electrical conductor coated with insulating enamel, a cotton serving around the enamel impregnated with a halogenated material, 30 and a braided outer covering of cotton treated with a flame-proofing material.
7. An insulated wire comprising a core covered with an insulating enamel, a cotton serving impregnated with a mixture of 35 chlorinated naphthalene and a relatively small amount of a bituminous material, and an outer covering of braided cotton treated with ammonium phosphate.

In witness whereof, we hereunto subscribe 40 our names this 25th day of November, A. D. 1925.

FRANK LOUIS ROMAN.  
HARRY THOMAS WINSEMIUS.